

## UNITED STATES PATENT OFFICE

RUSSELL MCGILL, OF WILMINGTON, DELAWARE, ASSIGNOR TO E. I. DU PONT DE NEMOURS & COMPANY, OF WILMINGTON, DELAWARE, A CORPORATION OF DELAWARE

## STABILIZATION OF ORGANIC NITRATES

No Drawing.

Application filed June 3, 1930. Serial No. 459,119.

This invention relates to a process for stabilizing organic nitrates.

In the co-pending application of Dr. James H. Werntz there is described a method of stabilizing organic nitrates by treating them with ethylene oxide. If the nitrate to be stabilized is a solid, this process is preferably carried out by dissolving it in a suitable solvent and treating it with ethylene oxide at temperatures at which ethylene oxide is a liquid. At temperatures at which ethylene oxide is a gas the treatment is carried out by bubbling the ethylene oxide through the nitrate. If the nitrate is a liquid, it is unnecessary to dissolve it. The use of ethylene oxide has the possible disadvantage that after the treatment the ethylene oxide, being gaseous at normal temperatures, will be volatilized and leave the organic nitrate. Should the organic nitrate subsequently be exposed to conditions which would tend to add or to generate unstabilizing decomposition products, the stability of the compound would be affected.

It is an object of this invention to stabilize organic nitrates. Another object of this invention is to stabilize organic nitrates by substances which are non-volatile at ordinary temperatures.

These objects are accomplished by stabilizing the nitrate with compounds which contain the ethylene oxide grouping and which have boiling points so sufficiently high that they will remain in the nitrate at ordinary temperatures. These objects are attained more particularly by the use of epichlorohydrin.

In the practice of my invention the nitrate to be stabilized, if solid, is preferably dissolved and treated with epichlorohydrin, although it may be treated with the epichlorohydrin without dissolving. After the treatment with epichlorohydrin the nitrate may be separated from the solution in any con-

venient way such as by precipitation with a non-solvent, or by distillation at low temperature and reduced pressure.

If the nitrate to be stabilized is a liquid, the epichlorohydrin is simply added thereto in sufficient quantities to attain the desired result.

Should it become desirable to stabilize a gaseous nitrate (for instance, methyl nitrate above 55° C.) the nitrate can be bubbled through the epichlorohydrin.

Should it be desired to remove the stabilizing agent and the product of its reaction with the unstabilizing compound, this can be done by washing the nitrate with water.

This invention is not limited to the use of epichlorohydrin but includes within its scope all compounds having the ethylene oxide group which have a boiling point sufficiently high to render them substantially non-volatile at ordinary temperatures. Among these compounds may be mentioned epiethylin (b. p. 129° C.), butadiene dioxide (b. p. 138° C.), epihydron alcohol (b. p. 162° C.), glycidic acetate (b. p. 169° C.), glycidic nitrate (b. p. 175° C.), and amyl epihydron ether (b. p. 188° C.).

The following examples illustrate the invention:

## Example I

A sample of glyceryl trinitrate, which had been washed several times with water and dried, was mixed with epichlorohydrin and its stability was determined by the Abel test. This test consists in heating a 1 g. sample of a nitrate at 65.5° C. in a test tube with a piece of starch-potassium iodide paper which has been wetted with a solution consisting of equal parts of water and glycerine. The appearance of a faint brown color on the paper indicates that the organic nitrate is decomposing. The number of minutes required for the appearance of color is noted in column two of the following table. In col-

85

90

95

100

umn three are given the percentages of epichlorohydrin added to the glyceryl trinitrate and in column four the number of minutes required for the appearance of color with epichlorohydrin. The test was stopped at the end of an hour in each instance and in no instance had decomposition of the treated samples been observed in that time.

| 10 | Column one          | Two                                                   | Three                    | Four                                                 |
|----|---------------------|-------------------------------------------------------|--------------------------|------------------------------------------------------|
| 15 |                     | Time for appearance of color before treatment—minutes | Per cent epichlorohydrin | Time for appearance of color after treatment—minutes |
|    | Glyceryl trinitrate | 35                                                    | 1.0                      | 60+                                                  |
|    | Glyceryl trinitrate | 35                                                    | 5.0                      | 60+                                                  |
|    | Glyceryl trinitrate | 35                                                    | 10.0                     | 60+                                                  |

### Example II

Three grams of mannitol hexanitrate was dissolved in epichlorohydrin after which the epichlorohydrin was evaporated and the mannitol hexanitrate washed with water and dried. The stability before treatment, as determined by the Abel test, was four minutes and after treatment was fourteen minutes.

My invention is applicable to the stabilization of other nitrates than those mentioned in the above examples, in fact to all organic nitrates which contain, or which may generate, unstabilizing decomposition products which are capable of reacting with the ethylene oxide radical. Among these organic nitrates may be mentioned cellulose nitrate.

Among the advantages of my invention is the fact that the stabilizing compounds remain in the nitrate and thus prevent its unstabilization by the addition or generation of unstabilizing compounds.

As many apparently widely different embodiments of this invention may be made without departing from the spirit and scope thereof, it is to be understood that I do not limit myself to the specific embodiments thereof except as defined in the appended claims.

I claim:

1. The method of stabilizing organic nitrates comprising adding thereto a substance containing the ethylene oxide structure having a boiling point so sufficiently high that it will remain in the compound.
2. The method of stabilizing organic nitrates comprising adding thereto a substance containing the ethylene oxide structure having a boiling point so sufficiently high that it will remain in the compound at ordinary temperatures.
3. The method of stabilizing organic nitrates comprising adding epichlorohydrin thereto.
4. The method of stabilizing organic ni-

trates comprising treating them with epichlorohydrin and removing the reaction products.

5. The method of stabilizing organic nitrates comprising treating them with epichlorohydrin and thereafter washing with water.

6. The method of stabilizing glyceryl trinitrate comprising treating it with epichlorohydrin.

In testimony whereof, I affix my signature.

RUSSELL MCGILL.

81

85

90

95

100

105

110

115

120

125

130